

May 19, 1959

C. A. BAER ET AL

2,887,419

COATING

Filed May 10, 1957



INVENTORS  
Wallace F. Bugbee  
BY Charles A. Baer  
Philip J. Clough  
Oliver W. Noyes  
ATTORNEY

1

2,887,419

## COATING

Charles A. Baer, Needham, Wallace F. Bugbee, Boston, and Philip J. Clough, Reading, Mass., assignors to National Research Corporation, Cambridge, Mass., a corporation of Massachusetts

Application May 10, 1957, Serial No. 658,919

9 Claims. (Cl. 148—6.35)

This invention relates to coating and more particularly to coating of black iron for the purpose of producing a "tin plate" substitute. This application is in part a continuation of application Serial No. 423,270, filed April 15, 1954, now abandoned.

The use of aluminum as a substitute for tin in the coating of black iron has long been the objective of numerous workers in the art due to the wide fluctuation in the availability and price of tin, particularly during times of war. Despite the great amount of research which has been done, it is believed that none of the prior workers has been successful. The principal reason for this has been a lack of appreciation of the fundamental requirements for an adherent, corrosion-resistant coating of aluminum on black iron.

Accordingly, it is a principal object of the present invention to provide an adherent, corrosion-resistant coating of aluminum on black iron.

Another object of the invention is to provide such a coating which is extremely thin, on the order of a few micro-inches in thickness.

Still another object is to provide such a coating which is applied to the black iron with vapor deposition techniques.

Still another object of the invention is to provide an improved article of manufacture.

Other objects of the invention will in part be obvious and will in part appear hereinafter.

For a fuller understanding of the nature and objects of the invention, reference should be had to the following detailed description taken in connection with the accompanying drawing which is a graph showing the time-temperature relationships forming a part of the present invention.

In a preferred embodiment of the present invention, black iron plate, after thorough cleaning, is passed through a vacuum chamber where a low pressure (on the order of 10 microns Hg abs. or less) is maintained. During passage through this chamber, the black iron is subjected to an aluminum vapor stream from a suitable source of aluminum vapors, such as shown in U.S. Patents 2,643,201 and 2,665,223. As described more fully hereinafter, the aluminum film deposited during the coating operation is not particularly adherent and certain precautions are taken in its manufacture to provide a rather porous film. The black iron having the porous aluminum coating is then passed out of the coating chamber and is given an aftertreatment comprising oxidation of the iron-aluminum interface at a temperature which is preferably maintained below the annealing temperature of the black iron. In a preferred embodiment of the invention, the aluminum-coated black iron is heated in an oxidizing atmosphere to a temperature above about 350° F. and below the annealing temperature of black iron (about 700° F.). At the upper temperature limits, the temperature need be maintained for only a few seconds, while at the lower temperature limits, particularly below 500° F., the tempera-

2

ture must be maintained for a time on the order of minutes rather than seconds. The product is maintained at this temperature for a time sufficiently long so that oxidation of the aluminum and iron at the iron-aluminum interface forms an adherent bond between the aluminum coating and the black iron plate. While the exact nature of this bond is not completely understood, it is believed to be an iron aluminate bond.

The drawing illustrates a graph which shows the relationship of time of heating to temperature of heating to obtain a satisfactory bond by oxidation. In this graph, the line A—B represents the very minimum time-at-temperature curve. Almost without exception, tests run below this curve A—B have failed to give a satisfactory bond. Tests run between curves A—B and C—D have given sporadically successful bonds, while tests run above curve C—D have been almost completely satisfactory.

It has also been discovered that the ability to form the adherent iron aluminate bond by oxidation after coating is a function of the coating conditions as well as the oxidation conditions. There are three principal factors to be considered in the formation of the initial aluminum coating. These are (a) the iron temperature during coating, (b) the temperature of the source of aluminum vapors, and (c) the distance traveled by the aluminum vapors from the source to the substrate. When the aluminum film is formed by depositing aluminum vapors which have traveled more than one mean free path from the aluminum source to the substrate, the resultant film is readily bonded with the base iron by subsequent oxidation treatment. On the other hand, an aluminum coating formed under conditions which permit deposition of aluminum vapors which have traveled less than one mean free path has been extremely difficult to bond by subsequent oxidation treatment. This is particularly true when the operation is carried out at near the limits for the other conditions specified above. For example, when the substrate is hot (e.g., near 200° F.) or the source is hot (e.g., 1600° C.), a coating applied at less than one mean free path can not be made adherent by subsequent oxidation treatment in any reasonable length of heating time.

The mean free path is the average distance which a molecule of gas travels before striking another molecule. It is given by the following equation:

$$\lambda = \frac{1}{\sqrt{2\pi n \bar{d}^2}}$$

$\lambda$  is the mean free path.

$n$  is the number of molecules per cubic cm.

$\bar{d}$  is the effective molecular diameter

The value for  $\bar{d}$  for aluminum given in the "Handbook of Chemistry and Physics" (31st edition, Chemical Rubber Publishing Company) is  $2.86 \times 10^{-8}$  cm. Using this value and the above equation at 1 micron Hg abs.,  $\lambda = 7.7$  cm. = 3.03 inches. Since the mean free path is inversely proportional to the pressure at low pressures, the following values can be calculated:

| P (microns Hg abs.) | Mean Free Path |      |
|---------------------|----------------|------|
|                     | Inches         | Cm.  |
| 0.1                 | 30.3           | 77.0 |
| 0.2                 | 15.2           | 38.5 |
| 0.5                 | 6.06           | 15.4 |
| 1.0                 | 3.03           | 7.7  |
| 2                   | 1.52           | 3.85 |
| 5                   | .60            | 1.54 |
| 10                  | .30            | .77  |

It is believed that the difficulty in obtaining a good bond by subsequent oxidation when the coating takes place

at less than the mean free path is due to the fact that the higher energy aluminum atoms encountered under these conditions form a denser coating. This denser coating is only slowly penetrated by the oxygen which is necessary to form the adherent bond. This same general problem arises if the temperature of the black iron is maintained above about 150° F. during the coating operation. This is particularly true when the aluminum vapor source has a high temperature on the order of 1600° C. In this case, the aluminum deposited on the heated substrate does not have sufficient adhesion by itself and its adhesion is difficult to improve by subsequent oxidative heat treatment. At low aluminum-vapor-source temperatures (e.g., 1200° C.), the substrate can be heated to a temperature as high as 300° F. without destroying the hardening effect of the later oxidation step. Accordingly, in a preferred form of the invention, the coating is carried out under conditions wherein (a) the aluminum vapors travel more than one mean free path from the source of aluminum vapors to the substrate and (b) the black iron substrate is maintained at a temperature below about 150° F. unless the aluminum vapor source temperature is relatively low such as 1200° C. or below.

#### Example I

A sheet of black iron 0.0095 inch thick was thoroughly cleaned and positioned in a vacuum chamber. The chamber was evacuated to a pressure on the order of .5 micron Hg abs. An aluminum-carrying filament spaced 11 inches from the black iron sheet was heated to a temperature of 1150° to 1200° C. to evaporate the aluminum. A coating of 16 microinches thick (as measured by electrical resistance) was deposited on the black iron, while the black iron was maintained at room temperature. The coated black iron was then removed from the coating chamber and the adhesion of the coating was tested by means of a pressure-sensitive adhesive tape and was found to be very poor. The coated black iron was then heated in air to 600° F. for 15 seconds. The adhesion was tested again and found to be excellent.

#### Example II

A sheet of black iron was treated as in Example I except that the coated black iron was heated in air to 500° F. for 1 minute. An excellent bond was formed between the aluminum and iron.

#### Example III

A sheet of black iron was treated as in Example I except that the coated black iron was heated at 500° F. in a vacuum (instead of air) for 5 minutes. The adhesion of the aluminum was still poor after the vacuum heat treatment.

#### Example IV

A sheet of black iron was treated as in Example I except that the black iron was heated to 200° F. during coating and the aluminum vapor source was at a temperature of about 1600° C. The adhesion of the aluminum was only mediocre and could not be improved by subsequent heating in air at 500° F. for 10 minutes.

#### Example V

A sheet of black iron was treated as in Example I except that the black iron was heated to 200° F. during coating. In this case, the aluminum vapor source was at about 1200° C. The adhesion of the aluminum coating was poor as removed from the coating chamber but became excellent after heating in air to 600° F. for 5 seconds.

#### Example VI

A sheet of black iron was treated as in Example I except that the black iron was only 6 inches away from the source of aluminum vapors. Since the pressure was .4 micron Hg abs., the black iron was less than one mean

free path from the source. The coating had only fair adhesion and was not appreciably improved by heating to 500° F. for 1 minute. After 3 minutes' heating at 500° F., the adhesion was satisfactory.

5 In the specification and claims, reference is made to the thickness of the aluminum film deposited on the black iron. Due to the extreme thinness of this film, its actual thickness cannot be readily measured. Accordingly, electrical resistance measurements have been used to obtain 10 calculated film thicknesses. The specific resistance of pure aluminum is  $2.8 \times 10^{-6}$  ohms per centimeter cube, thus, a centimeter square which is 0.1 micron=4 micro-inches=10<sup>-5</sup> cm. thick will have a resistance of

$$15 \frac{2.8 \times 10^{-6}}{10^{-5}} = 0.28 \text{ ohms per square}$$

$$16 \text{ microinch} \approx 1.12 \text{ ohms per square}$$

$$8 \text{ microinches} \approx 0.14 \text{ ohm per square}$$

$$16 \text{ microinches} \approx 0.07 \text{ ohm per square, etc.}$$

20 It should be remembered that thickness calculated from resistance measurement represents a minimum value. The actual thickness is undoubtedly greater in most cases since the calculation is based on two usually erroneous assumptions:

(1) That the film is completely continuous throughout its depth and is completely free of submicroscopic cracks so that resistance is at a minimum.

(2) That the film is packed to a maximum density.

30 While the invention has been particularly described in connection with its use for a "tin plate" substitute, it can be equally utilized for protecting ferrous objects in general.

Since certain changes may be made in the above process 35 and product without departing from the scope of the invention herein involved, it is intended that all matter contained in the above description shall be interpreted as illustrative and not in a limiting sense.

What is claimed is:

40 1. The process of producing a shiny, adherent, corrosion-resistant aluminum coating on black iron which comprises the steps of exposing black iron to a source of aluminum vapors in a vacuum chamber maintained at a pressure on the order of 10 microns Hg abs. and less to deposit on the black iron a film of aluminum having a thickness between about 1 to 30 microinches, and thereafter heating the aluminum-coated black iron in an oxidizing atmosphere at a temperature above about 350° F. and below about 700° F., said heating being continued 45 for at least a minimum time ranging between a few seconds at 700° F. to a few minutes at 350° F. and being sufficiently long to form an iron aluminate bond between the black iron and the thin aluminum coating.

50 2. The process of producing a shiny, adherent, corrosion-resistant coating on black iron which comprises the steps of exposing black iron to a source of aluminum vapors in a vacuum chamber maintained at a pressure on the order of 10 microns Hg abs. and less to deposit on the iron a film of aluminum having a thickness between about 1 to 30 microinches, the iron being maintained more than one mean free path of an aluminum molecule away from the aluminum vapor source during most of the time while it is exposed to the aluminum vapor source, and thereafter heating the aluminum-coated black iron in an oxidizing atmosphere at a temperature above about 350° F. and below about 700° F., said heating being continued for at least a minimum time ranging between a few seconds at 700° F. to a few minutes at 350° F. and being sufficiently long to form an adherent bond between the iron and the thin aluminum coating.

55 3. The process of claim 2 wherein the source of aluminum vapors is maintained at a temperature on the order of 1150° C. to 1200° C.

4. The process of claim 2 wherein the source of aluminum vapors is maintained at a temperature on the order

of 1400° C. and above and the black iron is maintained at a temperature below 150° F. during coating.

5. The process of producing a shiny, adherent, corrosion-resistant aluminum coating on black iron which comprises the steps of exposing black iron to a source of aluminum vapors in a vacuum chamber maintained at a pressure on the order of 10 microns Hg abs. and less to deposit on the iron a film of aluminum having a thickness between about 1 to 30 microinches, the iron being maintained more than one mean free path of an aluminum molecule away from the aluminum vapor source during most of the time while it is exposed to the aluminum vapor source and the iron being maintained at a sufficiently low temperature so that the resultant aluminum coating is relatively non-adherent, and thereafter heating the aluminum-coated black iron in an oxidizing atmosphere at a temperature above about 350° F. and below about 700° F., said heating being continued for at least a minimum time ranging between a few seconds at 700° F. to a few minutes at 350° F. and being sufficiently long to form an adherent bond between the iron and the thin aluminum coating.

6. The process of producing a tin plate substitute which comprises the steps of moving a strip of black iron past a source of aluminum vapors in a vacuum chamber maintained at a pressure on the order of 10 microns Hg abs. and less to deposit a thin, poorly adherent film of aluminum on the black iron, and thereafter heating the aluminum-coated black iron in an oxidizing atmosphere at a temperature above about 350° F. and below the annealing temperature of the black iron, the heating being continued for at least a minimum time ranging between a few seconds at temperatures as high as 500° F. and above to a few minutes at 350° F. and being sufficiently long to form an adherent iron aluminate bond between the black iron and the thin aluminum coating.

7. The process of producing a shiny, adherent, corrosion-resistant aluminum coating on black iron which comprises the steps of exposing black iron to a source of aluminum vapors in a vacuum chamber maintained at a pressure on the order of 5 microns Hg abs. and less to deposit on the iron a film of aluminum having a thickness between about 1 to 30 microinches, the iron being maintained more than one mean free path away of an aluminum molecule from the aluminum vapor source

during most of the time while it is exposed to the aluminum vapor source, and thereafter heating the aluminum-coated black iron in an oxidizing atmosphere at a temperature above about 350° F. and below about 700° F., said heating being continued for at least a minimum time ranging between a few seconds at 700° F. to a few minutes at 350° F. and being sufficiently long to form an adherent bond between the iron and the thin aluminum coating.

- 10 8. The process of producing a shiny, adherent, corrosion-resistant aluminum coating on black iron which comprises the steps of exposing black iron to a source of aluminum vapors in a vacuum chamber maintained at a pressure on the order of 1 micron Hg abs. and less to deposit on the iron a film of aluminum having a thickness between about 1 to 30 microinches, the iron being maintained more than one mean free path away of an aluminum molecule from the aluminum vapor source during most of the time while it is exposed to the aluminum vapor source, and thereafter heating the aluminum-coated black iron in an oxidizing atmosphere at a temperature above about 350° F. and below about 700° F., said heating being continued for at least a minimum time ranging between a few seconds at 700° F. to a few minutes at 350° F. and being sufficiently long to form an adherent bond between the iron and the thin aluminum coating.

- 15 9. A composite article of manufacture comprising an unannealed black iron sheet having a vacuum-deposited coating of aluminum thereon, the aluminum coating having a thickness on the order of 1 to 30 microinches, and forming a corrosion-resistant coating on said black iron which is superior to quarter-pound tin plate, the interface between the aluminum coating and the black iron having 20 been oxidized by heating to a temperature above 350° F. and below the annealing temperature in an oxidizing atmosphere to form an adherent iron aluminate bond therebetween.

40

References Cited in the file of this patent

UNITED STATES PATENTS

- 2,382,432 McManus et al. Aug. 14, 1945  
45 2,421,719 Simmons June 3, 1947